

## UNITED STATES PATENT OFFICE

1,962,172

## PROCESS OF NITRATING QUEBRACHITOL

Charles E. Burke and Russell McGill, Wilmington,  
Del., assignors to E. I. du Pont de Nemours &  
Company, Wilmington, Del., a corporation of  
Delaware

No Drawing. Application August 30, 1930,  
Serial No. 479,079

1 Claim. (Cl. 260—142)

This invention relates to new explosives and more particularly to an explosive compound produced by the nitration of quebrachitol, and also the method of producing an explosive compound 5 of this type. This invention also relates to explosive compounds containing in combination nitrated quebrachitol and nitrated polyhydric alcohols.

Quebrachitol (otherwise known as monomethyl 10 cyclohexanehexol or methyl ether of inositol) is a compound having the formula  $C_6H_{10}OCH_3(OH)_5$ , and occurs in appreciable quantities in rubber latex and at the present time is mostly discarded in solution in the serum after the rubber has been precipitated. It contains five hydroxyl groups as is indicated by the formula, and we have found that under proper conditions practically all of these groups can be nitrated, giving a compound which possesses excellent explosive properties.

On treating quebrachitol with nitrating acids, we have found that partial nitration may be effected with comparative ease, but that complete nitration can only be obtained by much more difficult procedure. We have found, however, that under proper conditions approximately complete nitration can be obtained and compounds showing a nitrogen value of from 95 to 100 per cent of the theoretical may be effected by our method.

While it will be apparent from this disclosure that quebrachitol pentanitrate may be prepared in various ways, we have found the following to be a preferred method, although it is to be understood that our invention is not limited thereto:

20 grams of finely ground quebrachitol is added slowly to 40 grams of 95% nitric acid, the temperature during this addition being maintained at approximately 10° C. 40 grams of concentrated sulfuric acid is then added to the nitric acid solution at such a rate that the temperature rises gradually to approximately 25° C., where it is maintained until all of the sulfuric acid has been added, after which it is agitated for one hour at approximately 25° C. in order to complete the nitration. The product is then allowed to separate from the spent acid and washed, neutralized and dried in the usual way. By this process a product has been obtained hav-

ing a nitrogen content only slightly below that of theory.

Quebrachitol pentanitrate prepared as above is a transparent viscous oil which is practically insoluble in water and spent acid. It is quite stable, and the sensitivity as determined by the drop test is somewhat less than one-half that of nitroglycerin.

In cases where quebrachitol pentanitrate can be used in combination with another ingredient in which it is soluble, the nitration can be considerably simplified by first mixing the ingredients and then nitrating the mixture. For example, a mixture of 25 grams of quebrachitol and 25 grams of ethylene glycol has been nitrated by adding the mixture to a slight excess of a mixed acid consisting of approximately 45% nitric and 55% sulfuric acid, at 10-15° C. In this nitration satisfactory results have been obtained by adding the mixture to the mixed acid in the course of half an hour, then agitating for an additional hour in order to complete the nitration. After the nitration is complete, the product is allowed to separate from the spent acid, and washed and neutralized in the usual way. This procedure gives a solution of quebrachitol pentanitrate in ethylene glycol dinitrate which is quite satisfactory for many purposes.

As an example of the way in which either quebrachitol pentanitrate alone or mixtures of this material with other ingredients, as mentioned above, can be used in the manufacture of propellant powders, the following illustration is given:

|                                                               | Parts |
|---------------------------------------------------------------|-------|
| Nitrocellulose                                                | 60    |
| Mixed quebrachitol pentanitrate and ethylene glycol dinitrate | 40    |
| Diphenylamine                                                 | 1     |

The nitrocellulose may be colloided by the other ingredients, using a volatile solvent if necessary and the powder finished by any of the procedures customarily used.

Mixtures of quebrachitol and glycerol may be nitrated in the same way as the mixture mentioned above and since the presence of the quebrachitol pentanitrate lowers the freezing point of the glycerol trinitrate the resulting combina-

tion is admirably suited for the preparation of low freezing dynamites.

As illustrative of one embodiment of our invention, and without in any way limiting it thereto, the following examples of compositions of low freezing dynamites are given:

1. A non-gelatinous dynamite.

|                       | Per cent |
|-----------------------|----------|
| 10 Nitroglycerin      | 34       |
| Nitrated quebrachitol | 6        |
| Sodium nitrate        | 46       |
| Wood pulp             | 10       |
| Sawdust               | 2        |
| Calcium carbonate     | 2        |
|                       | 100      |

15 2. A gelatinous dynamite.

|                       | Per cent |
|-----------------------|----------|
| 20 Nitroglycerin      | 27       |
| Nitrated quebrachitol | 5        |
| Nitrocotton           | 1        |
| Sodium nitrate        | 52       |
| Wood pulp             | 5        |
| Starch                | 8        |
| Calcium carbonate     | 2        |
|                       | 100      |

This invention also contemplates the nitration of quantities of quebrachitol together with solutions of carbohydrates and polyhydroxy alcohols having from four to six carbon atoms in liquid polyhydroxy alcohols. The carbohydrates may be either sucrose, glucose, or fructose, or other carbohydrates.

The polyhydric alcohols most satisfactory for our purpose are those containing from four to six carbon atoms. It is not necessary that each carbon atom contains a hydroxyl group. For ex-

ample, mannitol, sorbitol, dulcitol, ramnitol, arabitol, xylitol, pentaerythritol, erythritol, and other similar compounds may be used, although we preferably use sorbitol, or xylitol, or both in combination. Mixtures of any two, or of all these compounds may also be used with good results. A mixture of carbohydrate and hydrogenated carbohydrate aids in further lowering the freezing point of the finished explosive product.

The various compounds proposed in the foregoing may also be nitrated separately and then combined, although we have found it most desirable to combine the compounds before nitration.

By the term polyhydroxy alcohols having from four to six carbon atoms we purpose to include the sugars and also the polyglycerines and polyglycols.

It will be apparent from the foregoing that various embodiments of our invention exist and may be practiced within the scope thereof, and we do not intend to be limited except as indicated in the appended patent claim:

We claim:

The process of nitrating quebrachitol which comprises adding finely divided quebrachitol to nitric acid of approximately 95% strength, maintaining the temperature of the acid substantially constant during such addition, adding concentrated sulfuric acid to the nitric acid solution at such a rate as to give a gradual rise in temperature to 25° C.

CHARLES E. BURKE.  
RUSSELL McGILL.

35

110

40

115

45

120

50

125

55

130

60

135

65

140

70

145

75

150